



US005132170A

# United States Patent [19]

Terry

[11] Patent Number: 5,132,170

[45] Date of Patent: Jul. 21, 1992

## [54] RECHARGEABLE INKING MEMBER

[75] Inventor: Betty R. Terry, Weston, Conn.

[73] Assignee: Pitney Bowes Inc., Stamford, Conn.

[21] Appl. No.: 797,579

[22] Filed: Nov. 25, 1991

[51] Int. Cl.<sup>5</sup> ..... B32B 3/26[52] U.S. Cl. ..... 428/315.5; 428/315.7;  
428/315.9; 428/316.6; 428/317.1; 428/317.7;  
428/321.3[58] Field of Search ..... 428/315.5, 315.7, 315.9,  
428/316.6, 317.1, 317.7, 321.1, 321.3

## [56] References Cited

## U.S. PATENT DOCUMENTS

3,971,315 7/1976 Hansen ..... 428/315.5  
4,226,911 10/1980 Haren ..... 428/315.5  
4,336,767 6/1982 Wada ..... 428/315.5

5,006,404 4/1991 Terry ..... 428/316.6

Primary Examiner—William J. Van Balen  
Attorney, Agent, or Firm—Peter Vrahotes; Melvin J.  
Scolnick; David E. Pitchenik

## [57] ABSTRACT

A rechargeable ink pad having particular use with solution ink. The ink pad has a bottom layer of porous polychloroprene latex foam with pore sizes of 200 $\mu$  to 500 $\mu$  and a top layer of polyethylene foam with pore sizes of 10 $\mu$  to 20 $\mu$ . The two layers are secured to one another by a fusible web adhesive. A method of customizing the porous polychloroprene latex layer to obtain desired properties by felting has been discovered. Such felting renders the finished porous polychloroprene latex foam suitable for controlled ink flow required for printing purposes.

5 Claims, 2 Drawing Sheets





FIG. 2



**FIG. 3****FIG. 4**

## RECHARGEABLE INKING MEMBER

## COPENDING APPLICATION

Attention is directed to copending U.S. patent application Ser. No. 07/459,613 filed Jan. 2, 1990 and entitled Sustained Release Ink Dispenser, and concurrently filed patent applications entitled Method of Producing a Felted Porous Polychloroprene Latex Foam, by Betty R. Terry, Method of Shaping and Felting Open Cell Polychloroprene Latex Foam by Donald R. Allred and William S. Moller, and Method of Felting Open Cell Polychloroprene Latex Foam in Reduced Time by Donald R. Allred.

## BACKGROUND OF THE INVENTION

In the printing industry, there are generally two types of inks, dispersion inks and solution inks. Dispersion inks have been widely used throughout the years because they more easily can be formulated. The primary disadvantage of dispersion inks is that their components tend to settle and, as a result, the inks must be agitated on occasion. Although solution inks do not have a settling problem, they are more difficult to produce. Recently, strides have been made in the capability of producing solution inks, but such inks to have been found to be incompatible with the systems that are used to apply inks. For example, in the printhead of a postage meter, an inking pad or roller, hereafter collectively referred to as inking member, will contact the printhead to transfer ink thereto and the inking member will be removed from the printhead so that the inked printhead can contact a mailpiece to print an indicia.

There are also two general types of inking members, rechargeable inking members and self containing inking members. In developing solution inks, it has been found that inking members that are acceptable for use with dispersion inks simply are not efficient when used with solution inks. This is because inking members suitable for dispersion inks have pores that are too large. Such large pore sizes are required to allow dispersed particles to be distributed through the inking member. Additionally, typical inking members for dispersion inks were found to be incompatible with polyglycols, a component of contemporary solution inks. Consequently, it has become evident that if the benefits offered by solution inks are to be realized, inking members must be developed that will enhance the use of such inks.

## SUMMARY OF THE INVENTION

A rechargeable printing member has been formulated that is compatible with solution inks. The ink member consists of three layers: a first layer of microporous polyethylene that contacts a printhead to transfer ink thereto, a second layer of fusible web adhesive, and a third layer of porous polychloroprene latex which serves as a reservoir layer for ink. The third layer is formed as a felted porous polychloroprene latex foam material. With such an inking member, one obtains high quality indicia printing, excellent compatibility with solution inks, durability, and a high edge acuity.

Having the layer of porous polychloroprene latex foam felted was thought to offer particular advantages; however, no prior method of felting such a material was known. For this reason, a method was developed for felting porous polychloroprene latex which involves

placing the material under pressure then heating between 400 to 460° F. for a period of five to ten minutes.

## BRIEF DESCRIPTION OF THE DRAWINGS

- 5 FIG. 1 is a perspective, partially exploded view of an inking member made in accordance with the instant invention and the environment in which such an inking member is used;
- 10 FIG. 2 is a plan view of the inking member shown in FIG. 1 taken along the lines 2—2;
- 15 FIG. 3 is a cross sectional view of the inking member shown in FIG. 1; and
- 20 FIG. 4 is a cross sectioned view of a portion of an apparatus used to felt foam materials.

## 15 DETAILED DESCRIPTION OF THE PREFERRED EMBODIMENT

A portion of an inking system in which the present invention can be used is shown generally at 10 that includes an inking member 12. A tray 14 receives the inking member as will be described in greater detail hereafter. Inking systems 10 of the type in which the invention can be practiced are generally known, see for example U.S. Pat. No. 4,945,831, and will, therefore, not be described in detail. Although the invention is described as it applies to an inking pad, it will be appropriate that the invention applies equally as well to inking rollers without departing from the invention and the term inking member is intended to include inking pads, inking rollers or any other convenient forms.

The tray 14 has an ink distribution chamber 16 that has a plurality of laterally extending ribs 18 that form channels 20 therebetween. The tray 14 has an inlet nozzle 22 having a central opening 24 that is confluent with the ink distribution chamber 16 whereby ink can be supplied to the chamber by attaching a tube (not shown) to the nozzle 22 with the tube being attached to an ink supply (not shown). Optionally, an outlet ink nozzle 28 can be supplied to the tray 14 with the outlet ink nozzle 28 having a central opening 30 therein that is confluent with the ink distribution chamber 16. A tube (not shown) can be attached to the outlet nozzle 28 thereby allowing ink to be circulated through the ink distribution chamber 16. Also, with the presence of the inlet nozzle 22 and outlet nozzle 28 the ink distribution chamber can be cleaned with any appropriate cleaning fluid as required.

A pair of arms 34 located and attached to opposite ends of the tray 14 provide support for movement of the tray. A plate 38 having a central opening 40 therein is attached to the tray 14 and the central opening forms a part of the ink distribution chamber 16. A frame 41 is formed at the inner perimeter of the plate 3 and overhangs the ink distribution chamber 16 so that a portion of the inking member 12 is received between the frame and the chamber whereas the central portion of the inking member is exposed. Much of what has been shown and described thus far has been disclosed in U.S. Pat. No. 4,945,831, which also discloses an inker module in which the inking member 12 of the instant invention can be used. The manner in which the ink distribution chamber 16 is supplied ink and the manner in which the ink member 12 contacts a printhead is described in U.S. Pat. No. 4,945,831 and will not be described herein as the same does not form part of the instant invention.

The inking member 12 includes a first, or lower porous, layer 42, an upper, or second, porous layer 44 and an adhesive 46 therebetween to secure the first layer to

the second layer. The adhesive 46 is applied in the form of filaments that accumulate and cross over one another to form openings between the filaments. The thusly applied adhesive 46 creates a random non woven opening pattern that allows free flow of ink from the first layer 42 that serves as an ink reservoir to the second layer 44 that serves as a metering member. It will be noted that the first layer 42 is somewhat larger than the second layer 44 and that the frame 41 fits over the exposed portion of the first layer 42 and the second layer 44 is received in the opening 40 when the inking member 12 is received within the ink distribution chamber 16.

The first, or lower, layer 42 is preferably made of porous, also referred to as open cell, polychloroprene latex foam material having a pore size of 200 to 500 microns and serves as a reservoir of ink. Preferably, the polychloroprene latex foam material is felted and a manner in which it can be felted will be described hereinafter. The adhesive material that binds the two layers 42, 44 is a fusible web adhesive such as polyamide that is available from Freudenberg Nonwovens, Limited Partnership of Germany under the tradename PELLON. The second layer is a microporous sintered polyethylene having a pore size of about 10 to 20 microns. This second layer serves to meter ink to a printhead upon contact therewith.

The inking member 12 of the instant invention was made in the following manner. To achieve the right balance between resilience, conformance and re-inking ability, the polychloroprene latex foam layer 42 was felted 2:1. Since felting had not been performed on polychloroprene latex previously, felting conditions were developed using a high temperature press shown generally at 46, available from pasadena Hydraulics Inc., Model No. 950R18122S. The essential elements of a high temperature press is shown in FIG. 4 and includes an upper movable platen 50 which is attached to a piston 48 and a lower stationary platen 52. A source of heat 56 is provided in the form of resistive heating to heat the platens 50, 52 with foam material 60 to be felted located between the upper platen 50 and lower platen 52. A shim 54 is shown located on the lower platen 52. A number of important parameters had to be considered when determining processing conditions and feasibility of 15 felting. Included in the variables were initial foam 60 thickness, shim 54 thickness for control of pressure, felting ratio, initial density, press temperature and time. A foam of an initial thickness 60 was placed in the press and shims selected that would achieve the final felting ratio. Pressure was applied to the foam 60 with the initial thickness until contact was made between the upper platen 50 and the shim 54 resulting in the foam of reduced volume 62. For example, for a felting ratio of 2:1 and a finished polychloroprene latex thickness of 0.145", a press temperature of 400°-425° F., a time of 5-10 minutes, shim thickness of 0.15-0.140" and a pressure between 11,000 and 3,000 lbs/in<sup>2</sup>, with a foam starting thickness of 0.29" was found advantageous. For higher felting ratios, higher press temperatures or pre-heating are useful, but it should be noted that volume reduction is paramount in determining the degree of felting. Shim thickness depends on the desired felting ratio as well as final pad thickness. The amount of felting achieved is proportional to the reduction of volume 65

of the foam 60. If a 2:1 felting ratio is desired, the foam 60 originally placed in the press 46 will have its volume reduced by one half with heat applied for the periods above given. The felting of the polychloroprene latex open celled foam materials directly reduced the effect of pore size as well as increased the compression strength of the elastomeric foam material. As printing tests subsequently showed, by felting the bottom layer 42, the inking member 12 conformance was improved along with compressibility and ink pooling.

Once a felted layer 42 of the proper dimension was produced, the same was laminated to the second layer 44. The goal of lamination is to assure intimate contact between the top layer 44 and the bottom layer 42 without impeding ink flow. Thus, an open web type of material was chosen. For example, a polyamide adhesive can be used to heat laminate the polychloroprene latex layer 42 to the polyethylene layer 44. A press temperature of 248° F. for a period of 3 minutes using appropriate shims is effective for lamination. The temperature for laminating can vary from 220° to 270° F. and the time can vary from 2 to 4 minutes and the pressure can vary between 4,500 and 5,500 lbs/in<sup>2</sup>.

An inking member having a top layer 44 made of polyethylene foam, a bottom layer of porous polychloroprene latex foam and a fusible web adhesive for connecting the two has been shown to be quite advantageous. As opposed to prior materials, such as those discussed in U.S. Pat. No. 4,945,831, superior inking properties were achieved with solution inks. The inking member 12 of the instant invention resulted in an estimated operating life of 1 to 2 years and a printing life cycle of 500,000 to one million when used with a solution ink. With a foam inking member made of polychloroprene latex, the volume of swell was found to be 1% as opposed to 5.9% for prior materials. In addition superior print quality was achieved that directly correlates to the smoothness of the surface of the top layer 44 in which pore size is a factor. The smooth top surface provides excellent undistorted ink transfer to the printing plate it contacts for subsequent transfer of ink to paper. In addition, for the purpose of constant print intensity over continuous printing cycles, a dual layer composite must be used which combines a small pore size metering surface 44 and an open pore size storage layer 42 for long term continuous printing. This is accomplished with the instant invention.

What is claimed is:

1. A rechargeable inking member comprising: a first layer of porous, sintered polyethylene material having pore sizes of about 10-20 microns and a second layer secured to the first layer, the second layer being made of open cell polychloroprene latex foam material having pore sizes of 200-500 microns.
2. The inking member of claim 1 wherein said second layer is made of felted polychloroprene latex foam material.
3. The inking member of claim 2 wherein the degree of felting is 2:1.
4. The inking member of claim 1 wherein said first layer is attached to said second layer by a polyamide adhesive.
5. The inking member of claim 4 wherein said polyamide is in the form of a fusible web.

\* \* \* \* \*